# EUROPEAN PATENT SPECIFICATION

(11) **EP 0 013 186 B1**
(45) Date of publication and mention of the grant of the patent: **07.12.1983**
(21) Application number: 79303081.8
(22) Date of filing: 31.12.1979
(51) Int. Cl.: D01D 5/30, D01D 5/24

(54) **Process for melt-spinning a splittable conjugate filament; self-texturing splittable conjugate filament; and method of splitting such a filament**
Verfahren zum Schmelzspinnen eines spaltbaren konjugierten Filamentes, selbstkräuselndes spaltbares konjugiertes Filament; Verfahren zum Spalten eines solchen Filamentes
Procédé de filage par fusion d'un filament conjugué susceptible de se fendre; filament conjugué, à frisure latente, susceptible de se fendre; procédé de refente d'un tel filament

(30) Priority: 02.01.1979 US 848
(43) Date of publication of application: 09.07.1980
(62) Divisional of application: 82105614.0
(73) Proprietor: MONSANTO COMPANY, St. Louis, Missouri 63167 (US)
(72) Inventor: YU, Jing-peir, Pensacola Florida 32504 (US); Bromley, James Ernest, Pensacola Florida 32504 (US)
(74) Representative: McLean, Peter

## Description

The invention relates to the art of conjugate filaments splittable into sub-filaments. More particularly, it relates to a process and product wherein the conjugate filament itself has no substantial texture while sub-filaments splittable therefrom have substantial latent torqueless helical crimp.

Conjugate filaments splittable into sub-filaments are known to the art, as typified by Hayashi U.S. Patent 4,051,287. As disclosed therein, alternating segments of polyamide and polyester are spun in a side-by-side adhering relationship to form a hollow filament splittable into sub-filaments. Such sub-filaments can be of smaller denier than can be conveniently spun as separate filaments, lending a soft hand to fabrics made therefrom. The sub-filaments of Hayashi are not disclosed as possessing significant crimp, and, as illustrated in Figure 10 of the patent, are substantially flat (untextured) even though the conjugate filament had been textured by the false-twist heat-set method before being split into sub-filaments.

Tanner U.S. Patent 3,117,906 describes a process comprising generally preparing a grey fabric from yarn comprising composite filaments comprising at least two different synthetic polymeric components adhered together in side-by-side relation throughout substantially the entire length of the filament, said different components having different shrinkage characteristics when subjected to heat; subjecting the fabric to a treatment involving controlled conditions whereby the different components are separated to form separate filaments and heating the fabric to effect shrinkage of the filaments, the heating being of sufficient duration and intensity to cause the filaments from the different synthetic polymeric compositions to shrink to a substantially different degree. The differential shrinkage causes the filaments that shrink less to be pulled into crimped and looped configurations and the fabric is thereby bulked, but the filaments do not themselves possess latent torqueless helical crimp.

The process of the present invention is one for melt-spinning a hollow conjugate filament, splittable into sub-filaments, from nylon 66 and polyethylene terephthalate polymers axially arranged in an adhering relationship, the process comprising:-
a. Extruding a hollow molten stream formed from axially extending segments of said polymers arranged alternately in side-by-side adhering relationship to form said hollow molten stream;
b. quenching said stream to form a filament; and
c. withdrawing said filaments from said molten stream at a given spinning speed, characterised in that said given spinning speed is sufficiently high and said quenching is sufficiently rapid that unicomponent sub-filaments split from said filament possess substantial latent torqueless helical crimp.

The invention also comprises a conjugate filament of nylon 66 and polyethylene terephthalate polymers axially arranged in an adhering relationship, sub-filaments of said filament being releasably attached to one another in a side-by-side relationship, and said filament being substantially free of crimp, characterised in that unicomponent sub-filaments split from said conjugate filament possess substantial latent torqueless helical crimp.

The invention also includes a method comprising splitting a conjugate filament according to the invention into unicomponent sub-filaments.

According to a preferred aspect of the filament of the invention, the filament is hollow.

Other aspects of the invention will in part appear hereinafter and will in part be obvious from the following detailed description taken together with the accompanying drawing, in which:
The Figure is a bottom plan view (looking up) of the preferred spinneret orifice used in practising the invention.

As shown in the Figure, the preferred spinneret construction includes several generally arched or horseshoe-shaped slots 20 in spinneret blank 22 arranged symmetrically about a central point, the open ends of the horseshoe shape facing inwardly. The several slots 20 constitute a combined orifice for spinning a single filament. Slots 20 extend entirely through blank 22 except for a recessed web region 24 at the apex of each slot 20. The two dissimilar polymers are fed to the combined orifice as a sheath-core stream, with dotted circle 26 representing the interface between the two polymers. The adjacent ends of adjacent slots 20 are sufficiently close that the streams issuing therefrom unite just below the spinneret. The molten stream is thus a hollow structure composed of alternating axially extending segments of the two polymers. Surface tension and other effects tend to make the molten stream approach a hollow circular cross-section prior to solidification, substantially as shown in Hayashi Figure 1.

Each polymer segment accordingly has a portion of its periphery exposed to quenching on the exterior of the hollow stream, and an opposite portion shielded and not so exposed since it lies in the interior. According to the invention, the molten steam is exposed while under the stress of spinning to quenching sufficiently rapid as to produce substantial latent torqueless helical crimp in the sub-filaments splittable from the conjugate filament.

### Example I (Comparative)

Nylon 66 polymer and polyethylene terephthalate polymer, each of normal molecular weight for apparel end uses, are extruded at a temperature of 290°C through the combined orifice, the nylon polymer being the core of the sheath-core stream approaching the combined orifice. Equal volumes of the two polymers are supplied, with the extrusion rate selected to produce a conjugate filament having a denier of 19.5 at a spinning speed of 1500 yards (about 1350 meters) per minute. A quench zone just beneath the spinneret and 1 t meters in height is supplied with quenching air at 20°C, the air being directed horizontally onto the polymer stream and having a speed of 25 meters per minute. Below the quench zone, steam is applied to the filament, a conventional finish is applied, and the filament is wound.

The spun filament is then drawn at 65 meters per minute and at a draw ratio of 2.16 over a contact heater at 132°C, the heater being 0.4 meters long. The resulting drawn yarn, when mechanically worked to break the conjugate filament into 12 sub-filaments, develops no substantial torqueless helical crimp when subjected to boiling water.

### Example II

Example I is repeated, except that the spinning speed is increased to 4500 meters per minute while the denier of the conjugate filament is reduced to 4. The resulting sub-filaments, after separation and immersion in boiling water, form a highly voluminous and lofty yarn. Fabrics formed from the conjugate yarn acquire a very soft hand and increased bulk and covering power when the fabric is mechanically worked enough to separate the yarn into sub-filaments. Simple exposure of the fabric to boiling water is adequate in many instances, since the flexing of the yarn involved in certain fabric formations separates the sub-filaments.

## Claims

1. A process for melt-spinning a hollow conjugate filament, splittable into sub-filaments, from nylon 66 and polyethylene terephthalate polymers axially arranged in an adhering relationship, the process comprising:-
a. extruding a hollow molten stream formed from axially extending segments of said polymers arranged alternately in side-by-side adhering relationship to form said hollow molten stream;
b. quenching said stream to form a filament; and
c. withdrawing said filament from said molten stream, at a given spinning speed, characterised in that said given spinning speed is sufficiently high and said quenching is sufficiently rapid that unicomponent sub-filaments split from said filament possess substantial latent torqueless helical crimp.

2. A conjugate filament of nylon 66 and polyethylene terephthalate polymers axially arranged in an adhering relationship, sub-filaments of said filament being releasably attached to one another in a side-by-side relationship, and said filament being substantially free of crimp, characterised in that unicomponent sub-filaments split from said conjugate filament possess substantial latent torqueless helical crimp.

3. A filament defined in Claim 2, wherein said filament is hollow.

4. A method comprising splitting a conjugate filament defined in either of Claims 2 and 3 into unicomponent sub-filaments.

## Revendications

1. Procédé de filature par extrusion d'un filament conjugué creux, pouvant être dissocié en sous-filaments, à partir de polymères de nylon 66 et de téréphtalate de polyéthylène, disposés axialement en étant adhérents, comprenant les étapes suivantes:
a. l'extrusion d'un courant creux à l'état fondu, formé de segments s'étendant axialement des polymères placés alternativement côte à côte tout en adhérant de manière à constituer le courant creux à l'état fondu;
b. le refroidissement du courant de manière à former un filament; et
c. l'extraction du filament hors du courant à l'état fondu, à une vitesse de filature donnée; caractérisé en ce que la vitesse de filature donnée est suffisamment élevée et le refroidissement suffisamment rapide pour que des sous-filaments à un seul composant dissociés du filament possèdent un frisage hélicoïdal sans torsion sensiblement latent.

2. Filament conjugué de polymères de nylon 66 et de téréphtalate de polyéthylène, disposés axialement en étant adhérents, les sous-filaments du filament étant fixés de manière amovible les uns aux autres en étant côte à côte, et le filament étant sensiblement exempt de frisure, caractérisé en ce que les sous-filaments à un seul composant dissociés du filament conjugué possèdent une frisure hélicoïdale sans torsion sensiblement latente.

3. Filament selon la revendication 2, caractérisé en ce qu'il est creux.

4. Procédé comprenant la dissociation d'un filament conjugué défini dans l'une ou l'autre des revendications 2 et 3 pour donner des sous-filaments à seul composant.

## Patentansprüche

1. Verfahren zum Schmelzspinnen einer hohlen Zweikomponenten-Faser aus Nylon 66 und Polyethylenterephthalate-Polymeren die in aneinanderhaftender Beziehung angeordnet sind, die in Unterfilamente aufspaltbar ist, wobei das Verfahren die Massnahmen
a. Extrudieren eines hohlen geschmolzenen Stroms, der aus sich axial erstreckenden Segmenten der genannten Polymeren gebildet ist, die abwechselnd in aneinanderhaftender Seitean-Seite-Beziehung angeordnet sind, um den hohlen geschmolzenen Strom zu bilden;
b. rasches Abkühlen des Stromes zur Bildung einer Faser, und
c. Abziehen der Faser aus dem geschmolzenen Strom bei einer gegebenen Spinngeschwindigkeit, umfaßt, dadurch gekennzeichnet, daß die gegebene Spinngeschwindigkeit hoch genug ist und das Abkühlen hinreichend schnell erfolgt, daß die Einkomponenten-Unterfilamente, die von der Faser abgespalten werden, eine wesentliche latente drehmomentlose schraubenförmige Kräuselung aufweisen.

2. Zweikomponenten-Faser aus Nylon 66 und Polyethylenterephthalat-Polymeren, die axial in einer anhaftenden Beziehung angeordnet sind, wobei die Unterfilamente der Faser lösbar aneinander in einer Seite-an-Seite-Beziehung angeordnet sind, und die Faser im wesentlichen frei von Kräuselung ist, dadurch gekennzeichnet, daß die Einkomponenten-Filamente, die von der Zweikomponenten-Faser abgespalten werden, eine wesentliche latente drehmomentlose schraubenförmige Kräuselung aufweisen.

3. Faser nach Anspruch 2, dadurch gekennzeichnet, daß die Faser hohl ist.

4. Verfahren zum Aufspalten einer Zweikkomponenten-Faser gemäß einem der Ansprüche 2 und 3 in Einkomponenten-Unterfilamente.
